

June 21, 1932.

G. W. ELMEN

1,864,054

MAGNETIC MATERIAL

Filed July 29, 1926



Inventor:  
Gustaf W. Elmen  
W. Briggs  
Attorney

## UNITED STATES PATENT OFFICE

GUSTAF W. ELMEN, OF LEONIA, NEW JERSEY, ASSIGNOR TO WESTERN ELECTRIC COMPANY, INCORPORATED, OF NEW YORK, N. Y., A CORPORATION OF NEW YORK

## MAGNETIC MATERIAL

Application filed July 29, 1926. Serial No. 125,697.

This invention relates to magnetic materials and electromagnetic systems. It has wide application and is especially useful where the impressed magnetizing forces are

5 small, as in signaling systems.

Among the important characteristics of the material of this invention are high permeability, especially at low magnetizing forces, small hysteresis and high resistivity.

10 As a material the invention has its embodiment in magnetic compositions containing manganese preferably with nickel and iron. The proportions of the ingredients and the treatment of the material may be varied to emphasize one or more of its characteristics.

This application is in part a continuation of application, Serial No. 48,188, filed August 5, 1925.

15 Magnetic materials have been variously employed in electrical systems for such purposes as the cores of loading coils, transformers, magnetic modulators, etc., and for tractive electromagnets, for dynamos, motors, telephone receivers, telegraph relays, etc.

20 Magnetic materials have also been employed for the continuous loading of signaling conductors, but, until recently, this use has been limited to relatively short cables for telephone purposes. Heretofore the magnetic materials

25 generally used for these purposes have been soft iron and silicon steel. Recently, however, alloys consisting chiefly of nickel and iron have been employed to great advantage, particularly in connection with signaling sys-

30 tems and apparatus, in which the magnetic forces involved seldom exceed .2 gauss. Such alloys and the method of producing them are disclosed in U. S. Patent 1,586,884, issued June 1, 1926 and in applicant's copending ap-

35 plication, referred to above.

The application referred to discloses a composition of nickel and iron with the addition of a third element, and having high permeability, small hysteresis and eddy current

40 losses, and high resistivity. Among the compositions mentioned is an alloy of nickel, iron and manganese. The present invention re-

45 lates to magnetic materials consisting chiefly of nickel and manganese, or nickel, iron and manganese, and having higher permeability

than iron at magnetizing forces of the order of .2 gauss or less and a lower hysteresis and eddy current loss and higher resistivity than iron.

55 The invention will be more clearly understood by reference to the accompanying drawing, in which:

Fig. 1 indicates the change in initial permeability of alloys containing nickel, iron and manganese when the manganese content and the iron content are varied and the nickel content is kept at approximately 78% of the nickel-iron-manganese content;

60 Fig. 2 indicates the change in maximum permeability of alloys containing nickel, iron and manganese when the manganese content and the iron content are varied and the nickel content is kept at approximately 78% of the nickel-iron-manganese content;

65 Fig. 3 shows the change in resistivity of these alloys with varying percentages of manganese;

70 Fig. 4 indicates the change in hysteresis loss with variations in the percentage of manganese present; and

75 Fig. 5 is a perspective view of a signaling conductor loaded with the magnetic material of this invention in the form of tape.

80 It is readily seen from the curve of Fig. 1 that the initial permeability of alloys containing about 78% nickel and varying amounts of iron and manganese decreases with increasing amounts of manganese. This curve was plotted from values obtained testing a large number of alloys of varying percentages of iron and manganese, the nickel being kept at about 78%. One of these alloys containing about 77% nickel, .75% manganese and the balance iron had an initial permeability of slightly over 7700, while for an alloy containing about 80% nickel and 20% manganese, the iron present being negligible, the initial permeability was slightly over 2000.

85 90 95 As shown in Fig. 2, the maximum permeability of these alloys also decreases as the percentage of manganese increases, but the rate of decrease in maximum permeability is greater for the lower percentages of manganese than the rate of decrease in the initial

permeability as shown in Fig. 1. These values vary from 65,000 to about 5,600 in nearly a straight line proportion from the .75% alloy to the 20% alloy. Particular attention is directed to the fact that an alloy composed of substantially 80% nickel and 20% manganese with substantially no iron, has a higher initial permeability and a higher maximum permeability than either nickel or manganese taken alone. So far as is known, this is the first instance of an alloy of nickel and manganese having magnetic characteristics of this order.

The curve of Fig. 3 shows the variation in resistivity with varying percentages of manganese for alloys containing about 78% nickel and the balance manganese and iron. In the case of an alloy containing about 80% nickel and 20% manganese, the resistivity is over 50 microhms per c. c., which property, together with its relatively high initial permeability, renders this material better than iron for use as a loading material for signaling conductors and for other uses where the magnetizing forces are small and the eddy current loss may be large, as in transformer and inductance coil cores.

A further advantage of the alloys of nickel and manganese and of nickel, iron and manganese is their very low hysteresis loss as compared with that of iron or silicon steel. The variations of hysteresis loss in these alloys with change in composition and with a flux density  $B = 5000$ , is shown in Fig. 4. For the alloys having less than about 10% manganese the hysteresis is approximately 80 ergs per cu. cm. per cycle. With higher percentages of manganese the hysteresis loss increases but is still considerably less than that of iron.

Although alloys containing about 78% nickel have been found to give the highest permeability and to be preferable for many purposes, these characteristics are not limited to alloys containing 78% nickel since, by decreasing the percentage of nickel in the material, alloys having a higher resistivity may be obtained although the initial permeability of such alloys is ordinarily decreased. Thus, for example, it has been found that an alloy comprising approximately 70% nickel, 20% iron and 10% manganese has an initial permeability of 3580 and a resistivity of 55.7 microhm-cms. For certain purposes, as in the case of loading material for signaling conductors, an alloy of this character may be preferable to one having a higher initial permeability but a lower resistivity.

In preparing magnetic materials according to this invention, nickel, iron and manganese or, in some cases, nickel and manganese alone, are fused together in the desired proportions in an induction furnace and then poured into molds and worked or formed into the desired shape for use. For continuously loaded con-

ductors a particularly suitable form of the alloy is that of tape about .006 inch thick and about .125 inch in width.

In order to give the alloy the desired characteristics, it is necessary to subject it to a process of heat treatment which will be dependent upon the composition of the alloy and upon the particular characteristics which it is desired to produce in the material. An example of this heat treatment is to heat the alloy to about 1100° C. and maintain it at that temperature for a period of approximately one hour and subsequently cool the material slowly. The rate of cooling and the temperature to which the material is heated may be determined by experiment in each case in order that those characteristics sought in the material may be produced to the desired degree. An average rate of cooling which has been found to be suitable is approximately five degrees per minute. The temperature to which the material is heated may be considerably lower than 1100° C. or in some cases it may be higher.

A modification of this heat treatment, which is preferable in some instances, is to reheat the alloy, after the initial heat treatment outlined above, to a temperature somewhat above its magnetic transition point. The material is then cooled to room temperature, past the magnetic transition point at a certain rate which should be determined with each alloy but which is preferably faster than that employed in an anneal but not so fast as to set up strains in the material due to uneven cooling throughout the body. If desired, the reheating of the alloy may be omitted and the cooling from 1100° C. may be carried out in two steps at two different rates of cooling, that is, cooling from 1100° C. to a temperature slightly above the magnetic transition point at one rate and from that point to room temperature at another rate.

When the material is to be used for the continuous loading of signaling conductors, it is first formed into tape having the dimensions stated above. This tape is produced by working the alloy into the form of a rod or bar by repeated steps of swaging and annealing. The bar is subsequently drawn down to the form of wire of about No. 20 B. & S. gauge, and passed between rollers whereby it is flattened into tape of the proper thickness. This tape is next passed through cutting rolls or discs which trim its edges squarely on both sides and give the tape a uniform width.

The stranded conductor shown in Fig. 5 comprises a central cylindrical wire 11, enveloped by a plurality of surrounds 12 which are shaped to fit together closely to form a cylindrical annulus about the central wire. The magnetic material 13, in the form of tape, is wrapped helically about the stranded

copper core as disclosed in U. S. Patent 1,586,887, issued June 1, 1926. When it is desired to use the loading material in the form of wire rather than tape, the drawing process as outlined above is continued until the wire has the desired dimensions. The taped conductor is then given its final heat treatment by drawing it lengthwise through an electric furnace of the muffle type having a horizontal iron heating tube extending through the furnace and projecting a considerable distance beyond. The furnace is maintained at the optimum temperature for the composition of the alloy being employed. The length of the pass through the heating tube and the rate at which the conductor is moved are chosen so as to produce the most desirable magnetic characteristics in the loaded conductor. After cooling, the conductor is insulated and formed into a cable in the usual manner.

It will be found that certain of these alloys are better suited for some particular uses than others, and that the characteristics of any alloy may be varied by giving the material different heat treatments. No attempt has therefore been made to give an exhaustive analysis of the characteristics of each composition but merely to point out generally the characteristic advantages and uses of certain alloys and suggest typical methods of producing the same, with the understanding and intention that other similar compositions and methods of production are comprised within the spirit and scope of the invention as described and claimed.

What is claimed is:

1. A magnetic material comprising substantial quantities of nickel and manganese as essential elements thereof and having higher permeability than iron at low magnetizing forces.
2. A magnetic material comprising substantial quantities of nickel, iron and manganese as essential elements thereof and having a higher permeability at low magnetizing forces than any one of its components taken by itself.
3. A magnetic material comprising nickel, iron and manganese as essential elements thereof and having a lower hysteresis loss than iron at a magnetic induction of 5000 lines per square centimeter.
4. A magnetic material comprising nickel, iron and manganese as essential elements thereof, in which the iron and manganese contents each are not more than 20% of the nickel-iron-manganese content.
5. A magnetic material consisting of not less than 70% nickel and the remainder manganese and iron.
6. A magnetic material consisting of not less than 70% nickel, a substantial amount of but not more than 20% manganese and the remainder iron.

7. A magnetic material consisting of about 78% nickel and the remainder iron and manganese and having higher initial permeability than iron.

8. A magnetic material comprising nickel and manganese as essential elements thereof and having a higher permeability than iron at low magnetizing forces and in combination therewith an electrical conductor in inductive relation with said material for setting up magnetizing forces of a few tenths of a gauss or less therein.

9. A magnetic material consisting of not less than 70% nickel, a substantial amount of but not more than 20% manganese and the remainder iron and in combination therewith an electrical conductor in inductive relation with said material.

10. A transmission line continuously loaded with a magnetic material consisting of nickel, iron and manganese.

11. A loaded conductor comprising a conducting core and a layer of loading material wrapped helically thereabout, said loading material being chiefly composed of nickel, iron and manganese, the nickel comprising not less than 70% of the whole, the manganese comprising not more than 20% of the whole and the remainder iron.

12. A magnetic material of high permeability at low magnetizing forces such as occur in the magnetic material of continuously loaded signaling conductors, of low coercive force, and high specific resistance, consisting of an alloy of nickel greater than about 40%, manganese from a small amount up to about 20%, and the balance chiefly iron.

13. A magnetic material comprising 60% to 85% nickel, 15% to 40% iron and 4% to 20% manganese.

14. A magnetic alloy of iron, nickel and manganese having an initial permeability greater than 2000 and a resistivity greater than 20 microhm-cms.

15. Magnetizable material consisting of a basic alloy of iron and nickel, wherein the nickel content amounts to at least 40% and to which alloy, manganese from 2% to 20% is added.

In witness whereof, I hereunto subscribe my name this 22nd day of July A. D., 1926.

GUSTAF W. ELMEN.